

Dec. 23, 1958

R. C. HALTER ET AL

2,865,839

PROCESS FOR IMPROVING THE QUALITY OF LUBRICATING OILS

Filed June 19, 1956

2 Sheets-Sheet 1



INVENTORS.  
Richard C. Halter,  
James R. Miller,  
BY

Carl G. Ries

ATTORNEY.

Dec. 23, 1958

R. C. HALTER ET AL

2,865,839

PROCESS FOR IMPROVING THE QUALITY OF LUBRICATING OILS

Filed June 19, 1956

2 Sheets-Sheet 2



FIG. 3.

INVENTORS.  
Richard C. Halter,  
James R. Miller,  
BY

*Carl H. Ries*

ATTORNEY.

## 1

2,865,839

**PROCESS FOR IMPROVING THE QUALITY OF LUBRICATING OILS**

Richard C. Halter and James R. Miller, Baytown, Tex., assignors, by mesne assignments, to Esso Research and Engineering Company, Elizabeth, N.J., a corporation of Delaware

Application June 19, 1956, Serial No. 592,275

8 Claims. (Cl. 208—96)

This application is directed to a method for producing improved quality lubricating oils.

This application is a continuation-in-part of U. S. application Serial No. 408,878 for Richard C. Halter and James R. Miller, filed February 8, 1954, and entitled "Production of Improved Quality Lubricating Oils."

In accordance with the present invention a lubricating oil distillate fraction is treated in a process in which the fraction is hydrogenated under mild conditions of hydrofining by passing it over a cobalt molybdate hydrogenation catalyst in the presence of hydrogen at a temperature within the range of 575° to 750° F. and the reacted product from this hydrofining reaction is separated from gas and at least a substantial portion thereof contacted with a selective solvent in a solvent extraction zone to form an extract phase and a raffinate phase, the raffinate phase being recovered as the desired improved quality lubricating oil.

The process of the present invention is particularly adapted for the treatment of lubricating oil distillate fractions derived from Mid-Continent type crude oils and from Coastal type crude oils of the United States. These types of crude oils are well known to the art. For a description of properties of Mid-Continent type crude oils and Coastal type crude oils see "Characteristics of Crude Oils Currently Produced in the United States," by Harold M. Smith, The Oil and Gas Journal, March 29, 1951, pages 308, 309, 310, 313, 315, 317 and 318. It is not known exactly why the procedure of the present invention results in substantially improved results particularly when applied to lubricating oil distillate fractions derived from Mid-Continent type crudes and Coastal type crudes. By way of explanation, it is postulated that these distillate lubricating oil fractions contain a non-aromatic fraction of relatively low viscosity index and relatively high bromine number which cannot be removed economically by solvent extraction. It is further postulated that in the process of the present invention the hydrofining step converts said fraction to form which either is a more desirable lubricating oil component or a form which may be removed more readily by solvent extraction of both. However, this is given only by way of possible explanation of the improved results obtained in the practice of the present invention and is not presented by way of limitation.

The practice of the present invention will now be described in greater detail in conjunction with the drawing in which:

Fig. 1 is in the form of a diagrammatic flow sheet illustrating the practice of the present invention when treating a lubricating oil fraction derived from a Coastal type crude oil.

Fig. 2 is in the form of a diagrammatic flow sheet

## 2

illustrating the practice of the present invention when treating a lubricating oil derived from a Mid-Continent type crude oil; and

Fig. 3 is in the form of a series of curves illustrating the improved results obtained in the practice of the present invention.

Turning now specifically to the drawing, and first to Fig. 1, a lubricating oil fraction derived from a Coastal type crude oil is withdrawn from stock tank 11 through line 12 and charged to a furnace type heater 13 where it is heated and then withdrawn through outlet line 14 at which point hydrogen is added thereto through hydrogen inlet line 15. The fraction, before the addition of hydrogen, is at such a temperature that the mixture has a reaction temperature within the range of 575° to 750° F. as it passes through the catalytic reaction zone 16 into which it is discharged from line 14.

The hydrogen added to the lubricating oil fraction through line 15 is in an amount within the range of 200 to 2000 standard cubic feet of hydrogen per barrel of said oil distillate.

Reaction zone 16 contains a hydrogenation catalyst. A suitable catalyst may consist of cobalt molybdate within the range of 5% to 25% by weight and silica-free alumina in an amount within the range of 95% to 75% by weight. As a specific example, the cobalt molybdate hydrogenation catalyst may have a composition which is 15% by weight of cobalt molybdate and 85% by weight of alumina. Other suitable hydrogenation catalysts for this process include: molybdena on alumina, such as 8 to 10%  $\text{MoO}_3$  on alumina, or nickel tungsten sulfide.

In reaction zone 16 the distillate fraction and hydrogen are passed over the catalyst at such a rate that the amount of said distillate fraction is within the range of  $\frac{1}{4}$  to 3 volumes per volume of catalyst per hour. It is preferred to have a reaction pressure within the range of 700 to 800 pounds per square inch and a temperature of reaction within the range of 575° to 750° F. and, more preferably, within the range of about 650° to 750° F. It will sometimes be found preferable to conduct the operation within the temperature range of 625° to 675° F.

From reaction zone 16 a liquid product containing dissolved gas and a small amount of low flash point liquid is removed through line 17 and passed to a separator-stripper vessel 18 where the dissolved gas is separated from the liquid fraction and is removed through outlet line 19. A low flash point lighter-than-lube liquid fraction is also stripped from the hydrogenated lubricating oil fraction and removed through outlet 20. The gas-free flash-corrected liquid fraction is removed from separator 18 through line 21 and passed to a solvent extraction zone 22 where it is separated into a raffinate fraction which is removed through outlet line 23 as the desired high quality lubricating oil fraction and an extract fraction which is removed through outlet line 24.

Any suitable solvent such as phenol, liquefied sulfur dioxide, furfural, etc. may be employed in accordance with conventional techniques in the solvent extraction zone 22 to provide the lubricating oil raffinate fraction 23. Phenol is a preferred selective solvent which is employed with particularly desirable results in a manner well known to those skilled in the art. By way of example, when the extraction step is conducted utilizing phenol as the selective solvent, such extraction step may be carried out at a temperature within the range of 110° to 250°

F. Liquefied sulfur dioxide may be used as a selective solvent, in which case the extraction step may be carried out at a temperature within the range of about 30° to 120° F. As a further example, when furfural is employed, the extraction step may be carried out at a temperature within the range of about 150° to about 300° F.

A flow sheet for the treatment of a lubricating oil fraction derived from a Mid-Continent type crude is shown in Fig. 2. In Fig. 2 a Mid-Continent type oil fraction is withdrawn from stock tank 31 by line 32 and passed through furnace 33. The heated oil is withdrawn through line 34 and hydrogen is added thereto from hydrogen inlet line 35, and the oil and hydrogen then pass to catalytic reaction zone 36. Liquid product with dissolved gas and a small amount of low flash point liquid is withdrawn from catalytic zone 36 by means of line 37. The liquid fraction containing dissolved gas is passed from line 37 to separator-stripper 38 where the gas is separated and removed through outlet line 39, the low flash point liquid through line 40 and the liquid phase free from gas and low flash point liquid is withdrawn through outlet line 41. The steps carried out in units 31 through 41 may be identical to the corresponding steps carried out in units 11 through 21 of Fig. 1 and in order to simplify the description, these conditions will not be specifically set out with regard to Fig. 2. However, in Fig. 2 the fraction withdrawn through line 41 contains an appreciable amount of wax and it is desirable to remove said wax prior to the solvent extraction step. For this reason the fraction in line 41 is passed to a dewaxing step 42 where it is separated into a wax fraction removed through line 43 and the dewaxed lubricating oil fraction which is removed through line 44. The dewaxing of waxy lubricating oils is conventional to the art. Any of the conventional means for dewaxing the oil, as by the use of solvents, may be employed. The dewaxed oil from line 44 is passed to a suitable solvent extraction zone 45 where it is separated into a raffinate fraction removed through outlet line 46 as the desired lubricating oil fraction and an extract fraction which is removed through outlet line 47. To realize the full advantage of this invention, if dewaxing is required, the dewaxing step must be carried out subsequent to the hydrogenation step. The sequence of operations after the hydrogenation step is not critical and may be selected to be most convenient to the operator. For example, the dewaxing step may precede or follow the solvent extraction step.

The advantages of the present invention will be further seen by reference to the following examples:

#### EXAMPLE I

5 Samples of lubricating oil distillates derived from Mid-Continent type crude known as Panhandle light motor oil were used as the charge stocks. The specifications for these oils are as follows:

|                       |               |
|-----------------------|---------------|
| Gravity, ° API        | 29° minimum.  |
| Flash, ° F            | 450° minimum. |
| Viscosity at 210, SSU | 54-58.        |
| Viscosity index       | 102° minimum. |
| Pour point, ° F       | 15° maximum.  |

10 A sample of this distillate oil known as Sample A and another sample known as Sample B were subjected to hydrofining conditions as follows:

Table I

|                                                  | Hydrofining Conditions | Sample A | Sample B |
|--------------------------------------------------|------------------------|----------|----------|
| Temperature, ° F                                 | 700                    | 700      |          |
| Pressure, p. s. i. g.                            | 750                    | 750      |          |
| Feed rate, V/V/hr.                               | 3.0                    | 1.0      |          |
| Inlet H <sub>2</sub> rate, S. C. F./Bbl. of feed | 300                    | 900      |          |
| Vol. Percent yield of Flash-Corrected Lube       | 99.0                   | 95.5     |          |
| Wt. Percent yield of Flash-Corrected Lube        | 98.1                   | 94.4     |          |
| Wt. Percent yield of Con.ensable Non-Lube        | 1.1                    | 3.7      |          |
| Wt. Percent yield of Gas                         | 0.8                    | 1.9      |          |

30 The flash-corrected lubricating oil products from the hydrofining of Table I were dewaxed at a temperature in the range of -5 to -10° F. using a 5/1 ratio of secondary butyl acetate solvent/oil.

35 Samples were then extracted with phenol. In carrying out this extraction, another sample, sample C, which had not been subjected to hydrofining, but which had been clay contacted at 400° F. for 30 minutes, was divided into three portions with one portion inspected as reported in column 7 and the other two portions phenol extracted and inspected as reported in columns 8 and 9 of the following Table II. The product resulting from the treatment of sample A of Table II was divided into three fractions with one fraction inspected as column 1 and the other fraction solvent extracted as columns 2 and 3 in the following Table II. The product resulting from the treatment of sample B of Table I was divided into three portions with one portion inspected as reported in column 4 and the other two portions phenol extracted and inspected as reported in columns 5 and 6 of the following Table II.

Table II

| Columns                                      | Sample A |      |      | Sample B |      |      | Sample C |      |      |
|----------------------------------------------|----------|------|------|----------|------|------|----------|------|------|
|                                              | 1        | 2    | 3    | 4        | 5    | 6    | 7        | 8    | 9    |
| <b>Extraction Conditions:</b>                |          |      |      |          |      |      |          |      |      |
| Vol. percent phenol treat                    | 135      | 187  |      | 124      | 195  |      |          | 106  | 200  |
| <b>Inspections:</b>                          |          |      |      |          |      |      |          |      |      |
| Raffinate or dewaxed feed—                   |          |      |      |          |      |      |          |      |      |
| Feed                                         |          |      |      | Feed     |      |      | Feed     |      |      |
| Gravity, ° API                               | 26.9     | 30.2 | 30.8 | 27.4     | 30.2 | 30.7 | 25.9     | 29.2 | 30.6 |
| Flash, O. C. ° F                             | 445      | 455  | 460  | 420      | 450  | 455  | 435      | 460  | 465  |
| Vis./100, SSU                                | 421      | 339  | 320  | 372      | 328  | 319  | 481      | 368  | 337  |
| Vis./210, SSU                                | 57       | 55.0 | 54.2 | 54.9     | 54.3 | 54.1 | 59.2     | 56.2 | 55.2 |
| Vis. Index                                   | 84       | 100  | 102  | 87       | 100  | 102  | 80       | 97   | 102  |
| Pour, ° F                                    | 5        | 10   | 10   | 5        | 5    | 5    | 0        | 10   | 10   |
| Cloud, ° F                                   | 10       | 16   | 15   | 10       | 12   | 14   | Too      | 12   | 12   |
| Color, Tag Robinson                          | 2½       | 9½   | 10   | 2½       | 10   | 10½  | Dark     | 9½   | 10   |
| Extraction Yield, Vol. Percent Based on Feed |          |      |      |          | 81.7 | 78.4 |          | 79.0 | 70.2 |

The advantage of hydrofining prior to solvent extraction is shown in Fig. 3 in which the yields reported in Table II are plotted in the form of a curve. By way of a simple example which may be derived from the curve of Fig. 3, if it be assumed that a 150 volume percent of phenol feed is used the volume percent raffinate yield without the preliminary hydrofining step is approximately 74% whereas with mild hydrofining the volume percent raffinate yield is increased to 78% and with severe hydrofining the yield is increased to approximately 81%.

### EXAMPLE 2

A lubricating oil distillate fraction derived from Coastal distillate having a viscosity of 100 SSU at 210° F. was used as the feed stock. This feed stock was divided into three fractions one of which was subjected to hydrofining with one volume of feed per volume of catalyst per hour at 700° F. temperature, a pressure of 750 pounds per square inch gauge and 1400 standard cubic feed of hydrogen per barrel of feed stock. The product from this hydrofining step was then subjected to phenol extraction as reported in column 2 in Table III, hereafter, while another sample which had not been hydrofined was subjected to phenol extraction as reported in column 1 in Table III hereafter. The third sample was subjected to no treatment and inspections of this sample are reported in column 3 of Table III hereafter:

Table III

| Column.....                             | 1                 | 2                                 | 3     |
|-----------------------------------------|-------------------|-----------------------------------|-------|
| Treatment.....                          | Phenol Extraction | Hydro-fined then Phenol Extracted | Feed  |
| Extraction Conditions:                  |                   |                                   |       |
| Treat, Vol. Percent.....                | 141               | 115                               | ----- |
| Temperature, ° F.—                      |                   |                                   |       |
| Tower Top.....                          | 183               | 184                               | ----- |
| Tower Bottom.....                       | 173               | 172                               | ----- |
| Percent H <sub>2</sub> O in Phenol..... | 4                 | 4                                 | ----- |
| Percent H <sub>2</sub> O Injection..... | 4                 | 4                                 | ----- |
| Inspections:                            |                   |                                   |       |
| Raffinate—                              |                   |                                   |       |
| Gr., ° API.....                         | 24.4              | 24.6                              | 21.1  |
| Vis./100, SSU.....                      | 1435              | 1300                              | 2513  |
| Vis./210, SSU.....                      | 92.6              | 87.6                              | 111.8 |
| V. I.....                               | 67                | 66                                | 43    |
| Extract—                                |                   |                                   |       |
| Vis./210, SSU.....                      | 710               | 355                               | ----- |
| Gr., ° API.....                         | 8.4               | 9.6                               | ----- |
| Yields (based on feed)—                 |                   |                                   |       |
| Extraction, Vol. Percent.....           | 81.0              | 86.6                              | ----- |
| Overall, Vol. Percent.....              | 177.8             | 284.9                             | ----- |

<sup>1</sup> 96% yield in clay contacting step.

<sup>2</sup> 98.0% yield in hydrofining step.

It will be seen that an overall yield of about 85% is obtained when following the procedure of the present invention of hydrofining and then phenol extraction as compared with an overall yield of about 78% when no hydrofining step is used.

### EXAMPLE 3

A lubricating oil fraction derived from a Coastal type crude oil and having 1000 SSU viscosity at 100° F. was used as the charge stock. This stock was divided into three fractions. The first was not treated but was inspected with the inspections reported in column 3 of Table IV hereafter. The second sample was phenol extracted with the conditions of phenol extraction and the inspections of the product reported in column 1 of Table IV hereafter, while the third fraction was treated in accordance with the present invention by hydrofining at a temperature of 700° F., pressure of 750 pounds per square inch, liquid space velocity of .5 v./v./hr. and an inlet hydrogen rate of 1000 standard cubic feet per barrel of feed, the product from this reaction having gas and low flash point liquid separated therefrom and then phenol extracted with the conditions of phenol extraction and in-

spections of the product from the phenol extraction step reported in column 2 of Table IV hereafter:

Table IV

| 5                                       | Charge Stock.....        | 1000 CD          |                                   |       |
|-----------------------------------------|--------------------------|------------------|-----------------------------------|-------|
|                                         |                          | 1                | 2                                 | 3     |
| 10                                      | Treatment.....           | Phenol Extracted | Hydro-fined then Phenol Extracted | Feed  |
|                                         |                          |                  |                                   |       |
| Extraction Conditions:                  |                          |                  |                                   |       |
| 15                                      | Treat, vol. Percent..... | 168              | 168                               | ----- |
| Temperature, ° F.—                      |                          |                  |                                   |       |
| Tower top.....                          | 170                      | 170              | -----                             |       |
| Tower bottom.....                       | 160                      | 160              | -----                             |       |
| Percent H <sub>2</sub> O injection..... | 2                        | 2                | -----                             |       |
| Percent H <sub>2</sub> O in phenol..... | 4                        | 4                | -----                             |       |
| Inspections:                            |                          |                  |                                   |       |
| 20                                      | Stripped Raffinate—      |                  |                                   |       |
| Gravity, ° API.....                     | 25.9                     | 28.0             | 21.3                              |       |
| Vis./100, SSU.....                      | 516                      | 502              | 1043                              |       |
| Vis./210, SSU.....                      | 58.6                     | 58.1             | 69.7                              |       |
| Vis. Index.....                         | 64.8                     | 65.4             | 22                                |       |
| 25                                      | Stripped Extract—        |                  |                                   |       |
| Gravity, ° API.....                     | 12.9                     | 14.1             | -----                             |       |
| Vis./210, SSU.....                      | 120                      | 90.6             | -----                             |       |
| Yields, Vol. Percent (based on feed)—   |                          |                  |                                   |       |
| Extraction.....                         | 66.6                     | 76.2             | -----                             |       |
| Overall.....                            | 66.6                     | 71.6             | -----                             |       |

It will be seen from results reported in Table IV that the practice of the present invention resulted in an overall yield of 71.6 whereas the overall yield obtained when the sample was phenol extracted was only 66.6.

One skilled in the art of preparing lubricating oils will appreciate the substantial advantage in the higher yields obtained by the practice of the present invention.

35 While specific examples have been given, it will be understood that said examples are given by way of illustration only and not by way of limitation.

We claim:

1. An improved process for treating a lubricating oil distillate fraction derived from a crude oil taken from the group consisting of Mid-Continent and Coastal type crude oils comprising the steps of hydrogenating said lubricating oil distillate fraction over a hydrogenation catalyst in the presence of hydrogen in an amount in 40 the range of from 200 to 2000 cubic feet per barrel of said oil distillate while passing the hydrogen and said fraction co-currently over said catalyst at a rate within the range of 1/4 to 3 volumes of said fraction per volume of catalyst per hour at a pressure in the range of 700 to 800 pounds per square inch and at a temperature within the range of 650 to 750° F. to form a liquid phase containing hydrogen light hydrocarbon and a small amount of low flash point liquid, subsequently separating the gas and low flash point liquid from said liquid phase 45 to form a gas-free, flash-corrected liquid lubricating oil phase, contacting at least a portion of the lubricating oil components of said liquid lubricating oil phase with phenol in a solvent extraction zone to form an extract phase and a raffinate phase and recovering the raffinate phase as product.

2. A process in accordance with claim 1 in which the lubricating oil distillate fraction is derived from a Mid-Continent type crude oil and in which gas-free, flash-corrected liquid lubricating oil phase is dewaxed to form 55 a dewaxed oil fraction and said dewaxed oil fraction is the material contacted with phenol in the solvent extraction zone.

3. A process in accordance with claim 1 in which the lubricating oil distillate fraction is derived from a Coastal type crude.

4. An improved process for treating a lubricating oil distillate fraction derived from a crude oil taken from the group consisting of Mid-Continent and Coastal type crude oils comprising the steps of hydrogenating said lubricating oil distillate fraction over a hydrogenation

catalyst having approximately 15% by weight of cobalt molybdate and 85% by weight of aluminum in the presence of hydrogen in an amount in the range of from 200 to 2000 cubic feet per barrel of said oil distillate while passing the hydrogen and said fraction co-currently over said catalyst at a rate within the range of  $\frac{1}{4}$  to 3 volumes of said fraction per volume of catalyst per hour at a pressure in the range of 700 to 800 pounds per square inch and at a temperature within the range of 650° to 750° F. to form a liquid phase containing hydrogen, light hydrocarbon and a small amount of low flash point liquid, subsequently separating the gas and low flash point liquid from said liquid phase to form a gas-free, flash-corrected liquid lubricating oil phase, contacting at least a portion of the lubricating oil components of said liquid lubricating oil phase with phenol in a solvent extraction zone to form an extract phase and a raffinate phase and recovering the raffinate phase as product.

5. A process in accordance with claim 4 in which the lubricating oil distillate fraction is derived from a Mid-Continent type crude oil and in which said gas-free, flash-corrected liquid lubricating oil phase is dewaxed to obtain a dewaxed oil fraction and said dewaxed oil fraction is contacted with phenol in the solvent extraction zone.

6. A process in accordance with claim 4 in which the lubricating oil distillate fraction is derived from a Coastal type crude.

7. An improved process for treating a lubricating oil distillate fraction derived from a crude oil taken from

10  
15

the group consisting of Mid-Continent and Coastal type crude oils comprising the steps of hydrogenating said lubricating oil distillate fraction over a hydrogenation catalyst in the presence of hydrogen in an amount in the range of from 200 to 2000 cubic feet per barrel of said oil distillate while passing the hydrogen and said fraction co-currently over said catalyst at a rate within the range of  $\frac{1}{4}$  to 3 volumes of said fraction per volume of catalyst per hour at a pressure in the range of 700 to 800 pounds per square inch and at a temperature within the range of 575° to 750° F. to form a liquid phase containing hydrogen light hydrocarbon and a small amount of low flash point liquid, subsequently separating the gas and low flash point liquid from said liquid phase to form a gas-free, flash-corrected liquid lubricating oil phase, contacting at least a portion of the lubricating oil components of said liquid lubricating oil phase with a selective solvent under solvent extraction conditions in a solvent extraction zone to form an extract phase and a raffinate phase and recovering the raffinate phase as product.

20  
25  
30  
35

8. A process in accordance with claim 7 wherein the selective solvent is phenol.

#### References Cited in the file of this patent

#### UNITED STATES PATENTS

|           |               |       |               |
|-----------|---------------|-------|---------------|
| 2,660,552 | Blanding      | ----- | Nov. 24, 1953 |
| 2,687,982 | Baumann       | ----- | Aug. 31, 1954 |
| 2,701,783 | Long et al.   | ----- | Feb. 8, 1955  |
| 2,734,019 | Miller et al. | ----- | Feb. 7, 1956  |